

# UNITED STATES PATENT OFFICE.

WINFIELD S. POTTER, OF NEW YORK, N. Y., ASSIGNOR TO ALLOY STEEL FORGING COMPANY, OF WILMINGTON, DELAWARE, A CORPORATION OF DELAWARE.

## PRODUCTION OF MACHINED SHAPES OF MANGANESE STEEL.

1,018,366.

Specification of Letters Patent.

Patented Feb. 20, 1912.

No Drawing.

Application filed December 18, 1911. Serial No. 686,500.

*To all whom it may concern:*

Be it known that I, WINFIELD S. POTTER, a citizen of the United States, residing in the borough of Manhattan, city, county, 5 and State of New York, have invented certain new and useful Improvements in the Production of Machined Shapes of Manganese Steel; and I do hereby declare the following to be a full, clear, and exact description of the invention, such as will enable others skilled in the art to which it appertains to make and use the same.

My invention relates to the manufacture of cut gears or like shapes of manganese steel which require machining, such as pinions, bevel gears, spur gears, worms, threaded bars, and other machinery parts requiring accurate machining in addition to such forming as may readily be done by forging 20 or other hot shaping.

It has for its object the production of such manganese steel shapes in a condition of suitable hardness and strength, and of the requisite smoothness and accuracy of 25 finish in their machined portions.

As will hereinafter appear, the blank from which the cut gear or the like is to be made may be produced by rolling, forging, or pressing a suitably cast ingot of manganese 30 steel and cutting the same into individual blanks; or the blank may be cast to form, or cast nearly to form and subsequently wrought. In any case, the gears or the like, are brought into final form and condition 35 in an operation which consists of three main stages, to wit: a preliminary rough cutting of the teeth of the gear, at temperatures ranging from 500° C. upward, by means, for example, of a burring wheel or milling cutter of high speed steel; second, heat treating the roughly cut shape and quenching it so as to give it the desired toughness and strength; and completing the cutting at a 40 temperature of about 300° C. to 420° C. for the portions finally to be removed, the completion of the cutting being effected with a fine-toothed burring wheel, milling cut-

ter, reamer, or other tool of shape suitable for finishing the surfaces which require machining.

In the production of wrought manganese steel gear blanks or the like from an ingot, it is preferable to first cast the manganese steel ingot; then heat it until in a condition suitable for rolling; then roll it to a bloom 55 or billet, and cut off gear blanks of the desired weight. The blanks are brought into the desired form with an intermediate re-heating, if necessary, which may be at any temperature affording the requisite ductility 60 and which will usually range from about 800° C. to 1250° C. The blank should, however, in the final stage of the working operation be worked at temperatures between 800° C. and about 1075° C., so as to obtain 65 the preferred condition of the steel. The blank should then be heated to a red heat, say to between 500° C. and 1075° C. (preferably to about 900° C. to 1000° C.) for rough cutting to form, if such rough cutting is necessary. The rough cut shape is 70 then quenched, or first brought to an equalized temperature throughout of about 1000° C. and quenched; the equalizing reheat being of such a character as to again bring 75 into solution in the blank any carbids that may have separated out in the course of the operation. If the blank requires furthermore accurate machining, it should be heated, in the parts to be thus further machined, to about 300° C. to 420° C., and is then machined to finish, with suitable high speed steel tools. If extreme accuracy of 80 the finished shape is required, the blank is preferably evenly reheated throughout at 85 this time to a temperature between 300° C. and 420° C., and is then very rapidly cut to finished form, wherupon it is permitted to evenly cool to atmospheric temperature. In this manner, a distortion of the finished 90 shape by unequal shrinkage in cooling after the final machining is avoided. Additional accuracy in smoothness and finish may be obtained, in some cases, by grinding certain

parts of the piece to produce the desired surface.

Where the gear blank is to be cast as such, the manganese steel, of the desired composition, is cast into molds in such manner that porosity and shrinkage cavities are avoided in the cast blank. The blank is then separated from the gate and head metal, and is then heat treated either immediately from the heat of casting, or later, as desired, the purpose of this heat treatment being to bring into solution and even distribution throughout the mass, the carbids that have separated out during the freezing and cooling of the metal.

The cast gear blank may be brought into a wrought condition, at temperatures between 950° C. and 1250° C. by pressing or otherwise, and, in such case, should be finally worked at temperatures below 1075° C. and preferably at a temperature of about 1000° C. and should not thereafter be heated above 1025° C. for any considerable time of heating. For rough cutting the blank, it may then be brought to any temperature between 500° C. and 1075° C. and rough cut, and should then be quenched from a temperature substantially equalized throughout of from 800° C. to 1075° C. After quenching, it may then be reheated to between 300° C. and 420° C., for accurate machining, when such further machining is required.

In those instances in which the cast manganese steel blank is subjected to the preliminary cutting operation, without first pressing or otherwise working the blank, the preliminary cutting or machining operation is conducted, as above, at a temperature ranging from 500° C. to 1075° C., and when the preliminary cutting or machining required is so deep as to involve a heating to these temperatures (or to any temperature above 420° C.), a subsequent heat treatment will be necessary, consisting in bringing the metal to a temperature of about 1025° C. after the cutting operation, and for a time sufficient to restore the metal to a condition suitable for quenching. The cast blank may, in some instances, be heat-treated so as to bring into solution the carbids that have separated out during freezing and cooling; it may then be cooled, reheated to say 500° C. to 1075° C., and rough cut or machined at that temperature. It may then be heated to an equal temperature throughout within the range of say 975° C. to 1025° C. and immediately quenched. For final accurate machining, it may then be heated to between 300° C. and 420° C., machined to finished form, and finally cooled.

The method of making cut gears and other machined shapes in accordance with my invention, is characterized by the circumstance that after the blank has been

brought into a wrought condition, by suitable pressing, rolling or otherwise working it, before subjecting it to the cutting operation, the preliminary cutting is conducted under such conditions as not to destroy the wrought condition; furthermore, after the preliminarily cut blank has been quenched, the final accurate cutting is effected, in accordance with my invention, within a temperature range which will not destroy the toughness and hardness incident to quenching. These characteristic features are capable of utilization, either separately or in combination, as fully appears from the typical instances of the practice of the invention hereinbefore described.

Having thus described my invention what I claim is:

1. The method of producing machined shapes of manganese steel, which comprises working the metal at temperatures beginning at between 950° C. and 1250° C., continuing the working of the metal at temperatures between 800° C. and 1075° C. thereby obtaining a fine-grained wrought condition of the metal, preliminarily machining at temperatures between 500° C. and 1075° C., heating at temperatures between 800° C. and 1075° C., rapidly cooling to below 420° C. and completing the machining at temperatures between 300° C. and 420° C.; substantially as described.

2. The method of producing machined shapes of manganese steel, which comprises working the metal at temperatures which in the final forming are below 1075° C. and preserving the wrought condition incident to such working by machining at temperatures which are between 500° C. and 1075° C.; substantially as described.

3. The method of producing machined shapes of manganese steel, which comprises working the metal at temperatures which in the final forming are below 1075° C. and preserving the wrought condition incident to such working by machining at temperatures which are between 500° C. and 1075° C., and toughening the metal by heating at temperatures between 800° C. and 1075° C. and rapidly cooling to a temperature below 420° C.; substantially as described.

4. The method of producing machined shapes of manganese steel, which comprises working the metal at temperatures which in the final forming are below 1075° C. and preserving the wrought condition incident to such working by machining at temperatures which in the roughing stages are between 500° C. and 1075° C., toughening the metal by heating at temperatures between 800° C. and 1075° C. and rapidly cooling to a temperature below 420° C., and avoiding the loss of the toughened state by completing the machining at temperatures between

300° C. and 420° C.; substantially as described.

5. The method of producing machined shapes of manganese steel, which consists in heat-treating and working the blank until it is in a fine-grained toughened wrought condition, and avoiding loss of the toughened state during the final machining by effecting such final machining at temperatures be-

tween 300° C. and 420° C.; substantially as described.

In testimony whereof I affix my signature, in presence of two witnesses.

WINFIELD S. POTTER.

Witnesses:

JOHN C. PENNIE,  
MINERVA LOBEL.

Copies of this patent may be obtained for five cents each, by addressing the "Commissioner of Patents, Washington, D. C."